

Feb. 24, 1959

L. R. DUNN ET AL

2,875,044

FIBERBOARD AND METHOD OF FLAMEPROOFING THE SAME

Filed May 31, 1957



INVENTOR  
LEWIS R. DUNN  
LEWIS W. ECKERT

*Paul J. St. John*

ATTORNEY

1

2,875,044

## FIBERBOARD AND METHOD OF FLAME-PROOFING THE SAME

Lewis R. Dunn and Lewis W. Eckert, Lancaster Township, Lancaster County, Pa., assignors to Armstrong Cork Company, Lancaster, Pa., a corporation of Pennsylvania

Application May 31, 1957, Serial No. 662,698

12 Claims. (Cl. 92—3)

This invention relates to a fiberboard and method of flameproofing the same. It is concerned more particularly with the flameproofing of a cellulosic fiberboard such as one produced from wood fibers.

It has been proposed heretofore to flameproof fiberboard by applying to the surface thereof a coating consisting essentially of a mixture of borax and boric acid. The boric acid is primarily a glow inhibitor, and the borax serves chiefly to reduce flaming. The mixture of borax and boric acid provides a flame-resistant surface. It has been found, however, that the borax and boric acid coated board, when in service where it is exposed to conditions of relatively high humidity, is unsatisfactory, for the borax tends to bloom to the surface, affecting the appearance of the product and reducing its flame resistance.

Attempts have been made to overcome this problem by eliminating the borax, but the finished product is inadequate in flame resistance.

A cellulosic fiberboard product can be produced according to this invention which is resistant to blooming at high humidities and which is adequately resistant to flaming to meet United States Department of Commerce commercial standard specification CS-42-49, class F. This is accomplished by treating the surface of the cellulosic fiberboard, preferably while still in a wet condition prior to drying, with a solution of boric acid so that the same penetrates into the body of the board below the surface. The product is then heated to react the boric acid with the cellulosic fibers, preferably to a temperature of about 240° F. The dry product is then coated with a composition including clay or similar finely divided inorganic particles and a flame-resistant binder.

The felted fibrous body or board may be formed essentially from wood fibers. A wood fiberboard prepared as disclosed in Scott Patent 2,642,359 forms a suitable base or body. The fiberboard may be formed on a conventional fiberboard making machine, such as an Oliver forming machine. In this type of machine, a slurry of fibers suspended in water is deposited upon a rotating screen, and a continuous felted fibrous sheet is formed from which a portion of the water is extracted. The formed sheet is then delivered to a press, such as a Downingtown press, and additional water is removed from the sheet, and the sheet is consolidated to the desired thickness in the press.

The boric acid treatment may be effected by applying a solution of boric acid to the formed sheet as delivered from the Downingtown press in a wet condition, prior to drying. The coating may be applied by a roll coater, operating in advance of a pool of the boric acid solution which has been applied to the surface of the wet sheet.

In order to assist in the control of the penetration of the boric acid treating material into the wet board, a thickening agent such as sodium alginate or the like may be incorporated into the boric acid solution.

In the preparation of a suitable treating material, the

2

following ingredients are combined, all parts being given by weight:

|                                            |       |
|--------------------------------------------|-------|
| Boric acid                                 | 8.00  |
| Sodium alginate (Keltex sold by Kelco Co.) | 0.25  |
| Water                                      | 91.75 |

This provides an aqueous acid solution, the effective or active component of which consists essentially of boric acid.

10 In the preparation of the treating solution, the water is heated to about 140° F., and the powdered sodium alginate is stirred in for about 5 to 15 minutes, until a uniform distribution of it in the water has been obtained. Thereafter, the powdered boric acid is added, and the 15 mixture is stirred for about 5 minutes. The solution is maintained at a temperature of about 140° F. in order to insure that the boric acid will remain in solution. If the quantity of boric acid is substantially greater than 8%, then the temperature of the solution should be 20 maintained at a higher level in order to insure complete solution of the boric acid in the water.

25 The boric acid solution in heated condition is delivered to the surface of the fiberboard sheet; and the speed of movement of the sheet through the machine, the viscosity of the solution, the size of the pool applied behind the roll, and other variable factors affect the quantity of boric acid solution deposited onto the fiberboard and penetrating into the body thereof. Generally, a quantity equivalent to about 4 to 20 grams of boric

30 acid per square foot of fiberboard surface (on a dry weight basis) is adequate for the purposes of the present invention. A quantity equivalent to about 10 to 15 gram per square foot is preferred. The application of the heated boric acid solution to the wet surface of the 35 fiberboard (the board as delivered from the Downingtown press may have a surface temperature of about 100° F.) results in immediate interspersion of the boric acid treating solution and the water contained in the upper portion of the board; a slight penetration of the boric 40 acid solution into the body of the board occurs, the depth of penetration being controlled by the temperature of the solution, its viscosity, and other factors previously mentioned.

45 Due to this rapid interspersion of the boric acid solution into the top layer of the wet fiberboard, this wet-end application method is preferred. The same final results can, however, be obtained by applying the boric acid solution to a dried fiberboard sheet if provisions are made for adequate penetration of the solution, as 50 for example through the use of wetting agents with the moisture thus introduced into the dried fiberboard being subsequently removed by heat.

55 The surface treated board is then delivered to a conventional drier, and water is removed from the board and the boric acid reacts with the fibers in the area of penetration of the boric acid solution. In a typical drier installation, the first and middle zones may be heated to about 450° F. to 350° F. (from entrance to exit of each zone), and the exit zone may be similarly heated to about 370° F. to 260° F. It will be understood, of course, that until such time as substantially all of the water has been removed from the wet board, the temperature of the board will not exceed about 212° F.; and in the inner areas, the board temperature will be much lower. At completion of the drying operation, however, the board at the upper treated surface may be elevated to a temperature in the order of 220° F. to 250° F. The board drying temperatures and the duration of the drying time will vary with the thickness of the board, the quantity of water contained in the board at the time of delivery to the drier, the length of the drier zones, and other variable factors. The foregoing temperatures are

illustrative only. The treated surface of the board should be at some stage in the process elevated to a temperature of at least about 220° F. to insure an adequate reaction between the boric acid and the cellulosic fibers.

After the board has been dried, it is delivered to a work zone where a clay or equivalent top coat is applied, preferably in two stages; first, a thin prime coat and following that a finish coat. A suitable top coat may be formulated as follows, all parts being given by weight:

|                         |        |
|-------------------------|--------|
| Water                   | 1248.0 |
| Trisodium pyrophosphate | 3.0    |
| Clay                    | 1000.0 |
| Casein                  | 75.0   |
| Ammonia                 | 6.0    |
| Water                   | 16.0   |
| Pine oil                | 10.0   |

In the preparation of the coating composition, the trisodium pyrophosphate is dissolved in water and the clay is added. Mixing is continued until the clay is dispersed in the water. The trisodium pyrophosphate serves as a dispersing agent. Thereafter, the casein or other binder is added to the dispersion of clay and water, and mixing is continued. Following this, the ammonia, dissolved in the 16 parts of water, is added and mixing continued for a period of about two hours. The pine oil which serves as a wetting and leveling agent for the paint may be added at any convenient time during the process, and preferably during the mixing in of the ammonia treated casein solution.

Preferred practice is to apply the primer portion of the top coating by means of spray guns, followed by the application of heat and pressure to the surface by the use of heated ironing rolls. This tends to level the surface of the board by pressing down any projecting fibers which may extend above the surface. The heated rolls also elevate the temperature of the surface of the board, removing moisture from the prime coating. The ironing rolls may be heated by gas flames and have a surface temperature of about 900° F. They serve to elevate the temperature of the surface of the board to about 140° F. in a period of about one second.

The finish portion of the top coat may be of the same composition as the prime coat, and it may be applied by spray guns and then oven dried. Satisfactory results will be achieved if about 4 grams, dry weight, of the coating are applied per square foot of board surface in the prime coat and about 10 grams, dry weight, per square foot in the finish portion. The total quantity of clay or equivalent inorganic coating material applied over the boric acid treated layer will vary with the type of fiber in the board, the smoothness of the board texture, the size of the clay or other inorganic particles, and other variable factors. Preferably with a wood fiberboard such as discussed above a total of about 12 to 25 grams per square foot on a dry basis will be used. For practical purposes, about 30 grams per square foot is a reasonable upper limit, and as little as 4 grams will give some improvement with a smooth finished fiberboard.

An essentially complete covering of the inorganic particles over the boric acid treated layer of fibers appears to be desirable and is preferred. The exact action which occurs at the surface when the product is exposed to a flame is not understood. It has been observed in the making of fire tests of the product, however, that there is a confining action which seems to limit the spread of the flame. Regardless of theory, the fire tests prove that it is essential to have the inorganic coating of clay or the like disposed as a separate layer over the boric acid treated layer of fibers.

The nature of the chemical action involved between the boric acid and the wood fibers is not known. It has been found, however, that the combination of the boric acid treated layer of fibers and the clay layer disposed thereover provides a flame-resistant product which will

meet United States Department of Commerce commercial standard specification CS-42-49, effective November 15, 1949, and entitled "Structural Fiber Insulating Board," fourth edition, page 3, class F. The same product with the boric acid coating alone or the same product with a clay coating alone will not meet the specifications. Also, if the clay is combined with the boric acid solution and the two are applied as a single coating, the product does not meet the applicable specifications. In these respects, a dried fiberboard sheet treated with a boric acid solution so as to secure adequate penetration behaves in the same fashion as the wet-end treated material.

While it is preferred to apply the clay top coat after the board has been treated with the boric acid solution, heated, and dried, as mentioned above, it is possible to apply the clay coating as a so-called "wet-end" coating, subsequent to the application of the boric acid solution and after penetration of the boric acid solution below the surface of the board.

The following composition may be applied as a "wet-end" coating, all parts being given by weight:

|        |                                     |
|--------|-------------------------------------|
| Part A |                                     |
| 25     | Water ----- 912.0                   |
|        | Tetrasodium pyrophosphate ----- 3.3 |
|        | Fungicide (Dowicide G) ----- 3.0    |
|        | Klondike clay ----- 1100.0          |

|        |                                       |
|--------|---------------------------------------|
| Part B |                                       |
| 30     | Thin boiling starch (TSC) ----- 100.0 |
|        | Water ----- 268.0                     |
|        | Total solids about 50%.               |

In preparation of the composition, the starch and water of Part B are mixed and heated to about 190° F. to gel the starch. This gel is added to the clay slurry of Part A.

The mixture may be applied at room temperature to the wet board, after application of the boric acid solution and penetration of it below the surface of the board. It is preferred to use about 12 to 25 grams of this coating on a dry basis, over 10 to 15 grams of boric acid, also on a dry basis. A decorative coating may be applied and ironed onto the surface at the dry end, if desired, but is not necessary.

With a board  $\frac{3}{4}$ " thick and made of fiber such as disclosed in the Scott patent referred to, the penetration of the boric acid may be in the order of  $\frac{1}{16}$ ", and satisfactory results will be achieved. There is no critical limit to the depth of penetration of the boric acid treating solution, although for most purposes the thickness of the boric acid layer need not exceed about  $\frac{1}{16}$ " to  $\frac{1}{8}$ ". As mentioned previously, the dry weight of boric acid per square foot of board is preferably 10 to 15 grams, and the dry weight of clay or the like in the top coat is preferably 12 to 25 grams with a wood fiberboard made by the process of the Scott patent.

Where a thickening agent is used with the boric acid solution, the sodium alginate is preferred; but other thickening agents, such as carboxy methylcellulose, starch, and bentonite, may be substituted therefor as is well-known in the coating art. Generally, only a very small quantity of thickening agent will be used, in the order of 0.25% to 1.0% of the total weight of the treating solution.

In place of casein as the binder for the top coating composition, other binders may be used, such as antimony trioxide and chlorinated paraffin, polyvinyl acetate, and the like. They should, of course, be flame-resistant.

Calcium carbonate, atomite, whiting, lithopone, titanium dioxide, and the like and mixtures thereof may be substituted in whole or in part for the clay.

While the preferred base or body is a wood fiberboard, it is obvious that other similar products may be substituted therefor, such as fiberboards made from sugar

cane fibers, ground hard or soft wood, and other cellulosic materials.

A drawing is attached in which:

Figure 1 is a diagrammatic view which illustrates one method of carrying out the invention;

Figure 2 is a diagrammatic view which illustrates another method of carrying out the invention; and

Figure 3 is a diagrammatic view of a piece of fiberboard embodying the invention. The various elements of the product have been labeled in this view.

In the embodiment of the method shown in Figure 1, the wood fiberboard 2 is supported on rolls 3 and is delivered from a Downingtown press to a station 4 where a roll coater 5 applies the boric acid solution to the surface 6 of the board from a pool 7 disposed to the rear of the roll coater 5 in the direction of travel of the board as indicated by the arrow shown in the drawing.

As mentioned previously, preferred practice is to deliver the board thus treated with the boric acid solution to a drier for heating of the boric acid solution and drying of the board. (A break in the fiberboard 2 has been indicated in the drawing to diagrammatically illustrate this.) Thereafter, the top coating may be applied as shown in the drawing where the prime portion of the top coat is applied from a spray gun 8 to the surface and at the same time a coating is applied from a roll coater 9 to the bottom surface of the board in order to minimize the possibility of warpage. The prime coating applied to the surface is engaged by a heated ironing roll 10 which is traveling in the direction indicated by the arrow in the drawing, the same direction as the direction of movement of the board through the machine. The roll 10 is heated by a gas burner 11, and its surface temperature may be elevated to a high range, as noted previously. A corresponding ironing system may be applied to the under surface of the board. While a single ironing operation may be satisfactory, it is preferred to have two sets of ironing rolls, the second set of rolls being indicated at 12 in the drawing. They are heated by gas flame arrangements similar to the arrangement 11, and here too there is a lower ironing roll to compensate for the action of the upper roll and minimize warpage.

Spray guns 13 and 14 may be used to apply the finish portion of the top coat to the upper surface of the board. Since the lower surface has been set by the ironing operation, it is not necessary to apply any treating solution to the lower surface although a coating may be applied if desired. Thereafter, the material is delivered to a drier for final drying of the top coating.

In the embodiment of the method shown in Figure 2, the boric acid is applied to the surface of the fiberboard 2 in the same manner as in Figure 1; but in this embodiment, the top coat of clay is applied as a "wet-end" coating at station 15 where a roller coater 16 applies the coating composition previously mentioned to the surface 17 of the board from a pool 18 disposed to the rear of the roll coater 16 after the boric acid solution has been applied and has penetrated into the body of the wet board. A break has been indicated in the board to show an interval between the two roll coaters. With the top coating applied at the "wet end" to a wood fiberboard, preferred practice is to deposit over the boric acid treated surface about 20 to 25 grams per square foot of top coating material, on a dry basis. After application of the boric acid and the top coating, the board may be delivered to a conventional drier where water will be removed and the boric acid will be reacted with the cellulosic fibers. The drying temperatures may be those previously mentioned in connection with the drying of a fiberboard having a boric acid treating solution applied at the wet end.

The boric acid solution prevents discoloration of the board surface and thus permits the use of higher drying and reaction temperatures than would otherwise be possible. This is more fully disclosed in Eckert application,

Serial No. 519,256, filed June 30, 1955, and entitled "Method of Drying Water-Laid Fibrous Materials."

This application is a continuation-in-part of our pending application Serial No. 508,742, filed May 16, 5 1955, now abandoned, and entitled "Fiberboard and Method of Flameproofing the Same."

We claim:

1. In a process of rendering fiberboard and the like flame-resistant, the steps comprising forming a multiple 10 layer system on the upper surface of the fiberboard, including a layer made up of cellulosic fibers reacted with boric acid and a separate layer disposed thereover and made up of finely divided inorganic particles and a flame-resistant binder, by applying to the surface of a formed 15 body of felted cellulosic fibrous material an acid solution the active component of which consists essentially of boric acid, which solution penetrates only to a limited extent into the formed body below the surface thereof and said boric acid thus is concentrated in a surface layer 20 adjacent to the upper surface of the formed body, applying to the upper surface of the formed body over the boric acid coated fibers prior to drying a separate flame-resistant layer of finely divided inorganic particles and a flame-resistant binder, and at some stage in the process 25 heating the boric acid coated fibers to an elevated temperature at which said boric acid is reacted with said cellulosic fibers.
2. In a process of rendering fiberboard and the like flame-resistant, the steps comprising forming a multiple 30 layer system on the upper surface of the fiberboard, including a layer made up of cellulosic fibers reacted with boric acid and a separate layer disposed thereover and made up of finely divided inorganic particles and a flame-resistant binder, by applying to the surface of a formed body an acid solution the active component of which consists essentially of boric acid, which solution penetrates only to a limited extent into the formed body below the surface thereof and said boric acid thus is concentrated in a surface layer adjacent to the upper surface of the formed body, applying to the upper surface of the formed body over the boric acid coated fibers prior to drying a separate flame-resistant layer of finely divided inorganic particles and a flame-resistant binder, and at some stage in the process heating the boric acid coated fibers to an elevated temperature at which said boric acid is reacted with said cellulosic fibers.
3. In a process of rendering fiberboard and the like flame-resistant, the steps comprising forming a multiple 35 layer system on the upper surface of the fiberboard, including a layer made up of cellulosic fibers reacted with boric acid and a separate layer disposed thereover and made up of finely divided inorganic particles and a flame-resistant binder, by applying to the surface of a formed body an acid solution the active component of which consists essentially of boric acid, which solution penetrates only to a limited extent into the formed body below the surface thereof and said boric acid thus is concentrated in a surface layer adjacent to the upper surface of the formed body, applying to the upper surface of the formed body over the boric acid coated fibers prior to drying a separate flame-resistant layer of finely divided inorganic particles and a flame-resistant binder, and at some stage in the process heating the boric acid coated fibers to an elevated temperature at which reaction between said boric acid and said cellulosic fibers occurs, and forming over said surface layer a separate flame-resistant layer which consists essentially of finely divided inorganic particles and a flame-resistant binder.
4. In a process of rendering fiberboard and the like flame-resistant, the steps comprising forming a multiple 40 layer system on the upper surface of the fiberboard, including a layer made up of cellulosic fibers reacted with boric acid and a separate layer disposed thereover and made up of finely divided inorganic particles and a flame-resistant binder, by applying to the surface of a formed body an acid solution the active component of which consists essentially of boric acid, which solution penetrates only to a limited extent into the formed body below the surface thereof and said boric acid thus is concentrated in a surface layer adjacent to the upper surface of the formed body, heating said surface layer to a temperature at which reaction between said boric acid and said cellulosic fibers occurs, and forming over said surface layer a separate flame-resistant layer which consists essentially of finely divided inorganic particles and a flame-resistant binder.
5. In a process of rendering fiberboard and the like flame-resistant, the steps comprising forming a multiple 45 layer system on the upper surface of the fiberboard, including a layer made up of cellulosic fibers reacted with boric acid and a separate layer disposed thereover and made up of finely divided inorganic particles and a flame-resistant binder, by applying to the surface of a formed body an acid solution the active component of which consists essentially of boric acid, which solution penetrates only to a limited extent into the formed body below the surface thereof and said boric acid thus is concentrated in a surface layer adjacent to the upper surface of the formed body, heating said surface layer to a temperature above about 220° F. to react said boric acid with said cellulosic fibers in said surface layer, and forming over said surface layer a separate flame-resistant layer which consists essentially of finely divided inorganic particles and a flame-resistant binder.
6. In a process of fabricating a flame-resistant fiberboard, the steps comprising forming a slurry of felted cellulosic fibers into a sheet, removing a portion only of the water from the sheet, applying to the wet surface of the sheet an acid solution consisting essentially of boric acid and solvent therefor, which solution penetrates only to a limited extent into the formed body below the surface thereof and said boric acid thus is concentrated in a surface layer adjacent to the upper surface of the formed body in the amount of 4-20 grams per square foot, heating the formed body to a temperature of 220° F. to 250°

F. to react said boric acid with said cellulosic fibers in said surface layer, depositing as a separate layer over the surface layer a priming composition which consists essentially of finely divided inorganic particles and a flame-resistant binder therefor, heat and pressure ironing said surface coated with said priming composition to dispose within the body of the fiberboard projecting fibers which extend therefrom, and depositing a second coating of essentially the same composition as the priming composition over the ironed surface.

7. In a process of rendering fiberboard and the like flame-resistant, the steps comprising applying to the surface of a formed body of felted cellulosic fibrous material in wet condition an acid solution the active component of which consists essentially of boric acid, which solution penetrates only to a limited extent into the formed body below the surface thereof and said boric acid thus is concentrated in a surface layer adjacent to the upper surface of the formed body, applying to the upper surface of the formed body over the boric acid coated fibers in wet condition a separate flame-resistant layer of finely divided inorganic particles and a flame-resistant binder, and then heating said fiberboard product to an elevated temperature at which said fiberboard product is dried and said boric acid is reacted with said cellulosic fibers.

8. A flame-resistant fiberboard comprising a body of

cellulosic material carrying on one surface thereof and disposed within a limited area only of the body below said surface the dried residue of the heat reaction product of said cellulosic fibers and boric acid, and superimposed thereon and extending thereabove as a separate coat a layer of finely divided inorganic particles and a flame-resistant binder.

9. A flame-resistant fiberboard in accordance with claim 8 in which the finely divided particles comprise clay.

10. A flame-resistant fiberboard in accordance with claim 8 in which a casein binder is used in said separate coat.

11. A flame-resistant fiberboard in accordance with claim 8 in which the boric acid reacted fibers extend  $\frac{1}{8}$ " or less from the surface of the board.

12. A flame-resistant fiberboard comprising a body of cellulosic material carrying on one surface thereof and disposed within a limited area only of the body below said surface the dried residue of the heat reaction product of said cellulosic fibers an acid solution consisting essentially of boric acid and water, and superimposed thereon and extending thereabove as a separate coat a layer consisting essentially of finely divided inorganic particles and a flame-resistant binder therefor.

No references cited.